

## UNITED STATES PATENT OFFICE

2,221,597

## HEAT TREATING

Vincent T. Malcolm, Indian Orchard, Mass., assignor to The Chapman Valve Manufacturing Co., Indian Orchard, Mass., a corporation of Massachusetts

No Drawing. Application April 6, 1939,  
Serial No. 266,421

1 Claim. (Cl. 148—21.5)

This invention relates to improvements in heat-treating alloy steels and is directed more particularly to an improved process of heat-treating an alloy steel containing chromium, 5 tungsten, molybdenum, and vanadium in two or more combinations and the product of that process.

It is a principal object of the invention to provide a so-called alloy bolt steel to be used in high-pressure, high-temperature service where stability and creep resistance are of prime importance. That is to say, bolts or the like made from the steel of this invention are adapted to stand up under high pressures and temperatures as when 10 used in bolting flanges in various parts of high pressure and temperature equipment where leakage at joints must be prevented and where instability due to structural changes in the steel because of such high pressures and temperatures, 15 with consequent low creep resistance, has hitherto resulted in an inability of the bolts to maintain sufficient residual stress and, consequently, a tight joint.

Tests were made on various types of conventional steels with a newly developed relaxation machine to determine relaxation of the material under service conditions and to study the results of complete bolting set up in flanged joints. The result of this study showed unusual relaxation 20 and creep, together with structural changes in the steel itself.

As a special feature of this invention, my process produces bolts having structural constituents superior to those where ordinary heat treatments, 25 such as heating to critical transformation, quenching in liquid, and then tempering, are employed.

The ideal structure to attain in steel by means of any heat-treating processes is one of controlled grain without any visible network formation. In order to insure the absence of network 30 to a harmful degree, I have found as a result of much experimenting that prolonged heating at certain temperatures must be avoided and also, because of inherent sluggishness in steels, 35 that long soaking periods are desirable.

Accordingly, I provide the necessary soaking period without promoting undesired network formation by carrying out this portion of the treatment 40 at a temperature below the critical transformation point. In this way the steel may be brought to a uniform heat condition throughout, and be on the verge of recrystallization without danger of network formation. The soaking period I then follow by a normal period of heat-

ing above the critical transformation point to bring about complete recrystallization and grain size as desired by temperature adjustment in such a way that there is minimum opportunity for segregation to occur.

I then preferably cool the steel rapidly in air, because I have found that liquid quenching tends to be too drastic to maintain the desired structure. The drawing or tempering temperature is such that maximum strength and ductility for 10 the service intended are obtained and in the tempering operation the steel must be cooled slowly in the furnace to a temperature of below 500° F. in order to retain its properties, and to stop 15 secondary network formation.

For convenience this method will be termed "delayed heating" normalizing treatment, and the particular feature of this method which greatly influences the results obtained is the prenormalizing soak at a temperature below the 20 critical transformation point. I have found that thorough preheating of this kind seems to overcome the well recognized sluggishness in the 25 types of alloy steel with which I am concerned when the temperature of transformation is reached so that recrystallization takes place at a more normal rate of reaction which is important since sluggishness must be overcome if the tendency toward network formation is to be minimized.

One of the outstanding benefits of this treatment is the unusual uniformity of the physical properties of the steels when tested at room temperature and their ability to retain in great part these properties when in service in high 35 temperature and pressure installations. Steels treated according to my process have been tested for periods of time in temperatures up to 1000° F. and found to have retained their structure to the extent that it is directly comparable 40 with that of the material when it was placed in service.

From a standpoint of machineability, the extra hardness is compensated for by the fact that steels treated according to the process of this 45 invention lack appreciable network formation and are capable of being machined with greater ease. That is to say, a hardness of 360 Brinell in my specially treated steel will machine as readily as a hardness of 280 Brinell in the liquid 50 quenched steels.

I have experimented with various alloy steels in the development of this process, such as one containing, in addition to iron, of course, from 4 to 6% of chromium and either about 5% of

5 molybdenum, or 1% of tungsten, or a combination of .5% of molybdenum and 1.50% of silicon. Another alloy experimented with, contained from 1.75 to 2.25% chromium and about .5% molybdenum; another from .50 to 1.00% chromium and .5% molybdenum and .85 to 1.25% tungsten; still another from 1 to 1.50% of chromium, from 1.50 to 2.25% of tungsten, and from .20-.30% of vanadium.

10 As a result of this experimenting, I have developed a new alloy which has all of the desired characteristics above mentioned. This alloy has the following preferred formula, the stated proportions being approximate:

|                 | Per cent |
|-----------------|----------|
| Carbon          | .35-.55  |
| Manganese       | .40-.85  |
| Silicon         | .45-.75  |
| Chromium        | .90-1.25 |
| 20 Molybdenum   | .50-.65  |
| Vanadium        | .25-.35  |
| Phosphorus, max | .04      |
| Sulphur, max    | .04      |
| Iron            | Balance  |

The preferred process of heat treating this type of steel will now be described.

30 The piece or pieces are first heated slowly in a suitable furnace to about 1450° F. The heating is delayed at this point by allowing the steel to soak for about one and one-half hours for each inch of thickness.

Then the pieces are heated slowly to about 35 1550° F. and rapidly to 1750° F. Soaking at the rate of  $\frac{1}{2}$  hour for each inch of thickness is then continued, after which the steel is cooled rapidly in air.

40 After the cooling step, I reheat the pieces to 1250° F. for one and one-half hours for each inch of thickness. This is followed by slow cooling in the furnace to below 500° F. and again cooling in air.

45 Bolts processed according to this heat treatment have been used for high temperature and high pressure service with excellent results. Tests have shown that they have the following average physical properties:

|                                       |         |
|---------------------------------------|---------|
| 50 Tensile strength, lbs. per sq. in. | 172,350 |
| Yield point, lbs. per sq. in.         | 151,700 |
| Elongation in 2 inches, percent       | 17      |
| Reduction of area, percent            | 45      |
| Brinell hardness                      | 341     |
| Charpy impact ft. lbs. keyhole notch  | 15      |

55 These same newly-processed steels tested in temperatures up to 1000° F. for short periods of time show the following properties:

|                                       |         |
|---------------------------------------|---------|
| 60 Tensile strength, lbs. per sq. in. | 105,000 |
| Yield point, lbs. per sq. in.         | 85,000  |
| Elongation in 2 inches, percent       | 20      |
| Reduction of area, percent            | 62      |

65 Creep tests of this newly-processed steel made at 1000° F. for a period of not less than 5000 hours showed a creep limit of 22,000 pounds per square inch for 1% creep in 100,000 hours. Relaxation tests based on 60,000 pounds per square 70 inch initial stress at 950° F. showed residual stress of 20,000 pounds per square inch after 1000 hours.

The same steel above described when treated by a conventional process, that is heated to 1700° F., quenched in oil, drawn to 1250° F., and cooled

in air had the following physical properties as contrasted with those listed above:

|                                    |         |
|------------------------------------|---------|
| Tensile strength, lbs. per sq. in. | 145,000 |
| Yield point, lbs. per sq. in.      | 126,000 |
| Elongation in 2 inches, percent    | 17.5    |
| Reduction of area, percent         | 47      |
| Brinell                            | 310     |
| Charpy impact, ft. lbs.            | 16      |

When this same conventionally treated steel 10 was tested for a short time under temperature of 1000° F., it had the following properties as contrasted with the above-listed properties of my steel shown by the same test:

|                                    |        |
|------------------------------------|--------|
| Tensile strength, lbs. per sq. in. | 90,000 |
| Yield point, lbs. per sq. in.      | 65,000 |
| Elongation in 2 inches, percent    | 20     |
| Reduction of area                  | 65     |

Creep tests of this same conventionally-treated steel showed the following, as contrasted with what was stated above concerning steel treated according to this invention: creep limit at 1000° F. for a period of not less than 5,000 hours showed 25 a value of 10,000 lbs. per sq. in. for 1% creep in 1000 hours. Relaxation tests on steel treated according to the prior art based on 60,000 lbs. per sq. in. initial stress at 950° F. showed a residual stress of 9,000 lbs. per sq. in. in 1000 30 hours.

In my investigation a series of test pieces were heated for various periods of time at different temperatures in order to ascertain the structural changes which take place upon heat treatment. 35 Complete work on the several steels was carried out at various temperatures of from 1350° F. to 2150° F. and, at each temperature, for periods beginning with 5 minutes, then raising the time in increments of 10 minutes until one hour was reached, then in steps of 20 minutes until three 40 hours holding time was attained.

After each test for each period of time at each 45 temperature, recrystallization, diffusion, grain refinement, carbide segregation, and network formation were all noted and checked with critical transformations. Micro-sections and hardness determinations were taken of each specimen of each type of steel in each range at various times so that structures obtained could be critically 50 studied.

Prolonged heating at certain temperatures resulted in a change in grain size and a lack of any visible segregation. Above certain temperatures the network again appeared and persisted. 55

Steels containing this network formation are objectionable in that they show very little ductility in tension or bending, have low impact value, and are brittle wherefore they are of little value for high-temperature and/or high-pressure service.

The series of experiments just described showed that two conditions control the structural characteristics of such steels, namely temperature and time, and that of these, temperature is of 65 primary importance.

While I have described the invention in great detail and with respect to the present preferred form thereof, it is not desired to be limited thereto since changes and modifications may be made 70 therein without departing from the spirit and scope of the invention. The invention may be embodied in other specific forms without departing from the essential characteristics thereof. The present embodiments are therefore to

be considered in all respects as illustrative and not restrictive, the scope of the invention being indicated by the appended claim rather than by the foregoing description, and all changes which come within the meaning and range of equivalency of the claim are therefore intended to be embraced therein.

What it is desired to claim and secure by Letters Patent of the United States is:

10 The process of heat-treating alloy bolt steels of the pearlitic type of chromium steel to increase the creep resistance of the steels consisting of, preheating the steel by slowly soaking it at a

temperature below its critical transformation point for a period at the rate of about one and one-half hours for each inch of thickness of steel, following the soaking by a period of slow heating at a temperature above its critical transformation point for a period at a rate of about one-half hour for each inch of thickness, rapidly cooling the steel in air, then reheating the steel to a temperature below its critical transformation point for a period at a rate of about one and one-half hours for each inch of thickness, and then allowing the steel to cool slowly.

VINCENT T. MALCOLM.